

M. D. PHELAN,  
METHOD OF MAKING FORMS,  
APPLICATION FILED MAY 15, 1917.

1,290,338.

Patented Jan. 7, 1919.



Fig. 1.



Fig. 2.

Fig. 4.



INVENTOR.

Merton D. Phelan  
By his Attorney,  
Merton D. Phelan

# UNITED STATES PATENT OFFICE.

MERTON D. PHELAN, OF BOSTON, MASSACHUSETTS, ASSIGNOR, BY MESNE ASSIGNMENTS, TO UNITED SHOE MACHINERY CORPORATION, OF PATERSON, NEW JERSEY, A CORPORATION OF NEW JERSEY.

## METHOD OF MAKING FORMS.

1,290,338.

Specification of Letters Patent.

Patented Jan. 7, 1919.

Application filed May 15, 1917. Serial No. 168,839.

*To all whom it may concern:*

Be it known that I, MERTON D. PHELAN, a citizen of the United States, residing at Boston, in the county of Suffolk and State of Massachusetts, have invented certain Improvements in Methods of Making Forms, of which the following description, in connection with the accompanying drawings, is a specification, like reference characters on the drawings indicating like parts in the several figures.

This invention relates to a method of uniting two metals or alloys of different melting points and, in order to promote brevity, will be described as embodied in a method of making brass-faced iron forms for use in boot and shoe "sole-molding" machines.

In the manufacture of certain types of boots and shoes it is customary to shape the soles of the shoes by subjecting them while wet to a heavy pressure between suitably shaped forms. When these forms are made of iron and are allowed to come into direct contact with the soles a very objectionable black discoloration is produced due probably to the formation of iron tannate by the action of a solution of tannic acid in the leather upon the iron of the forms. It would, of course, be possible to obviate this undesirable result by making the forms of some other metal than iron, for example of brass, but the expense involved is almost if not quite prohibitive. The object of the present method is to produce a form the body of which is iron or other inexpensive metal or alloy but the operative portion of which is brass or other suitable alloy or metal, the brass portion or facing being of sufficient thickness and attached with sufficient strength to the iron to permit it to stand prolonged and severe use.

In the illustrative method a brass plate is placed in a mold and then molten iron is introduced into the mold whereby the brass is melted and remains molten after the iron has solidified. The plate is not flat but has high and low portions; and as a consequence of this and of the shrinkage which takes place as the iron solidifies, the brass tends to run down leaving one or more localities thinner than others. In one of its aspects the invention comprises a method of making a composite article of two materials having different melting points which consists

in placing in a mold a piece of the material having the lower melting point, pouring into contact with it molten material having the higher melting point whereby the material having the lower melting point is melted, and then pouring into the molten material having the lower melting point an additional amount of the same material. In the illustrative method an additional amount of molten brass is poured into the molten brass after the iron has solidified.

In another of its aspects the invention comprises a method such as that described above in which the piece or plate of the material having the lower melting point is suspended in the upper part of the mold and the molten material having the higher melting point is poured in from beneath.

These and other aspects of the invention will be set forth in connection with an illustrative apparatus by which the method may be practised.

Referring now to the accompanying drawings,—

Figure 1 shows a brass plate supported above a pair of Bunsen burners as it appears after having received its coating;

Fig. 2 shows an open molding box with the brass plate suspended in the upper portion of the mold;

Fig. 3 is a section in detail showing more particularly the manner in which the plate is suspended;

Fig. 4 is a vertical longitudinal section through the molding box after the brass and iron have solidified.

In carrying out the method of the present invention, a brass plate 5 is first provided having the desired shape except that two ears 7 project from its sides and are provided with threaded holes 9 to receive the threaded ends of rods 11. These rods have eyes at their upper ends through which extends a long rod 13 the ends of which rest upon wedges 15 laid upon the upper part of the molding box. By forcing the wedges 100 beneath the long rod 13 the brass plate may be held firmly in place as shown in Figs. 2 and 3.

Before, however, it is suspended or fastened in place as has been described, it receives the following treatment. First it is cleaned in any suitable manner, as for instance by being buffed. It is then laid on

- a suitable support such as the rods 19 and brought to and maintained at the desired temperature by any suitable heating apparatus such as the Bunsen burners 21.
- 5 While the plate is hot it is coated with solder on the side against which the molten iron will rise in the mold; then brass chips are dropped upon the pasty solder, then a little muriatic acid is sprinkled over the 10 chips and solder, and finally a coating of borax is dusted over the whole surface. The plate is then cooled, the solder acting to hold the chips and borax in place on the plate after the plate has been inverted and 15 suspended from the rod 13 in the upper part of the mold as shown in Fig. 2, the plate being embedded in and flush with the surface of the molding sand except at its rear portion. At the rear of the plate—that is 20 at the portion which is adjacent to the heel portion in the finished form—a hollow is formed in the sand as indicated by the line 23 so that the heel portion of the finished form will have an iron surface. This particular sort of form is, however, immaterial 25 so far as the present invention is concerned.
- In the lower half of the molding box is formed the lower portion of the mold 25 into which the molten iron is to be poured. This 30 lower portion has a core 27 extending into it to provide a slot to receive a bolt by which the form when finished may be fastened to a support in use. This core, however, and the particular shape given to the 35 heel portion of the form by it, is immaterial so far as the present invention is concerned and may be changed or dispensed with as may be desired. Leading out of the mold 25 are two channels 28 over parts of which 40 the ears 7 of the plate 5 lie when the molding box has been closed (see Fig. 3) and flow gates or sprues 29 lead upwardly from these channels. The ingate through which the molten iron enters the mold is indicated 45 at 31. The rods 11 extend through sprues or gates 33, 35 in the upper half of the mold of which one, for example 33, serves, as will presently be described, as an ingate and the other as a flow gate.
- 50 In practising the method the upper and lower parts of the molding box are fastened together in the usual manner after the plate 5 has been coated as described and fixed in place in the upper portion of the mold.
- 55 Molten iron is then poured down the ingate 31, flows into the bottom of the mold and rises in the mold and in the sprues 29. The heat of the iron melts the brass plate and maintains the brass in a molten condition for some time after the iron has solidified. The molten brass under these circumstances and owing to the shrinkage of the iron tends to flow down toward the ends of the mold, for example to the level of the broken line 60 A—A in Fig. 4 and it becomes necessary to

supply more brass to fill the space above this line. To this end the rods 11 are lifted out, and molten brass is poured down the sprue 33 and rises in the sprue 35. It will be understood that the location of the line 70 A—A in the drawing is purely arbitrary and has been used merely to indicate in a general way what would be the effect if no extra brass were added. The bond which is produced by this method between the 75 brass and iron possesses great strength, the metals apparently mingling more or less in their molten states and thus to an extent becoming embedded one in the other.

Having thus described my invention, I 80 claim as new and desire to secure by Letters Patent:

1. The method of making a form having an iron base and a brass working surface which consists in placing a brass plate in a 85 mold, pouring in molten iron whereby the brass is melted and remains molten after the iron adjacent to it has solidified, and then pouring into the molten brass an additional amount of the same material. 90

2. The method of making a form having an iron base and a brass working surface which consists in suspending a brass plate in the upper part of a mold, pouring in molten iron from beneath whereby the brass is 95 melted and remains molten after the upper portion of the iron has solidified, and then pouring in from the top a small amount of molten brass.

3. The method of making a form having 100 an iron base and a brass working surface which consists in applying to one face of a brass plate a coating comprising solder, small particles of a metal having a lower melting point than that of iron and a flux, 105 suspending the plate in the upper part of a mold with the coated face downward, and pouring in molten iron from beneath.

4. The method of making a form having 110 an iron base and a brass working surface which consists in applying to one face of a brass plate a coating comprising solder, small particles of a metal having a lower melting point than that of iron and a flux, 115 suspending the plate in the upper part of a mold with the coated face downward, pouring in molten iron from beneath, and then after the brass has melted pouring in from the top a small amount of molten brass.

5. The method of uniting a plate of brass 120 to a base of iron which consists in applying to one face of the plate a coating comprising solder, brass chips and a flux, suspending the plate in the upper part of a mold with the coated face downward, and pouring the iron 125 in from beneath.

6. The method of uniting a plate of brass to a base of iron which consists in applying to one face of the plate a coating comprising solder, brass chips and a flux, suspend- 130

ing the plate in the upper part of a mold with the coated face downward, pouring the iron in from beneath, and then after the brass has melted pouring in from the top 5 a small amount of molten brass.

7. The method of making a form having an iron base and a brass working surface which consists in heating a brass plate, applying to the plate while hot a coating comprising solder, brass chips and a flux, allowing the plate to cool, suspending the plate in a mold with the coated face downward, and pouring in molten iron from beneath.

8. The method of making a form having 15 an iron base and a brass working surface which consists in heating a brass plate, applying to the plate while hot a coating comprising solder, brass chips and a flux, allowing the plate to cool, suspending the plate in 20 a mold with the coated face downward, pouring in molten iron from beneath, and after the brass has melted, pouring in from the top a small amount of molten brass.

9. The method of making a metallic form 25 comprising a base and a working surface which consists in placing in a mold a plate of the material having the lower melting point, pouring in molten material of the higher melting point whereby the material 30 of the lower melting point is melted, and remains molten after the material of the higher melting has solidified, and then pouring into the molten material of the lower melting point an additional amount of the same 35 material.

10. The method of making a form having an iron base and a working face of an alloy of lower melting point than iron which con-

sists in suspending a plate of the alloy in the upper part of a mold, pouring in molten 40 iron from beneath whereby the alloy is melted and remains molten after the iron has solidified, and then pouring in from the top a small amount of molten alloy.

11. The method of making a form of two 45 materials having different melting points which consists in applying to one face of a plate of the material having the lower melting point, a coating of solder, placing the plate in a mold with the coated face exposed, 50 and pouring in molten material of the higher melting point.

12. The method of making a form of two materials having different melting points 55 which consists in applying to one face of a plate of the material having the lower melting point a coating of solder, placing the plate in a mold with the coated face exposed, pouring in molten material of the higher 60 melting point whereby the plate is melted and remains molten after the material of the higher melting point has solidified, and then pouring into the molten material of the lower melting point an additional amount of the 65 same material.

13. The method of making a composite article of two materials having different melting points which consists in placing in a mold a piece of the material having the lower melting point, pouring upon it molten material having the higher melting point, and then pouring in molten material having the lower melting point.

In testimony whereof I have signed my name to this specification.

MERTON D. PHELAN.